

June 3, 1930.

H. M. WILLIAMS

1,761,028

## HEATING FURNACE

Original Filed March 30, 1926



୧୩୫

Inventor

Harry M. Williams

Spencer, Hardman  
and Felt

his Attorneys

## UNITED STATES PATENT OFFICE

HARRY M. WILLIAMS, OF DAYTON, OHIO, ASSIGNOR TO GENERAL MOTORS RESEARCH CORPORATION, OF DETROIT, MICHIGAN, A CORPORATION OF DELAWARE

## HEATING FURNACE

Original application filed March 30, 1926, Serial No. 98,600. Divided and this application filed November 1, 1927. Serial No. 230,326.

This invention relates to the manufacture of porous metal articles such as shafts, bearings, or other objects which are used in rubbing contact with relatively moving metallic bodies. The porosity of the article is provided by a large number of minute voids or cells, which are connected by small capillary passages which render the body capable of absorbing substantial quantities of lubricant which is given out to the surface in contact with the relatively moving body.

The object of the present invention is to provide improvements in the apparatus used in the manufacture of porous metal bodies, in order to reduce the cost of the manufacture and to improve the quality of the product.

This application is a division of application Serial Number 98,600, filed March 30, 1926.

Further objects and advantages of the present invention will be apparent from the following description, reference being had to the accompanying drawings, wherein a preferred form of the present invention is clearly shown.

In the drawings:

Fig. 1 is a diagrammatic, longitudinal sectional view of a heat treating furnace used in the process of making porous metal articles according to the present invention.

Fig. 2 is a sectional view on the line 2—2 of Fig. 1.

The process of making porous metal bodies, to which the present invention relates, consists chiefly in mixing finely divided metals and graphite, in briquetting the mixture to form an article of the desired shape, and in heating the article in a non-oxidizing atmosphere and to a temperature sufficient to cause alloyage of the metallic ingredients. The graphite remains inert but spaces the particles of the alloyed metals, so that minute capillary passages are formed between the particles of graphite and particles of the alloyed grains or particles.

The porosity of the article is increased by using an organic volatile substance in the mixture of the metallic powders and graphite. This substance will escape during the heat treating process through crevices of the

crystals and alloyed particles, leaving minute voids which are connected by capillary passages. Beneficial results are obtained in some instances by the addition of a volatile flux which has the double function of assisting in the alloyage of the metallic particles and in increasing the porosity.

The following formula is typical:

|                   | Parts |
|-------------------|-------|
| Copper            | 90    |
| Tin               | 10    |
| Graphite          | 6     |
| Salicylic acid    | 2     |
| Ammonium chloride | 0.5   |

The proportions are by weight of the total mixture and the ingredients are mixed into a finely divided state. After mixing thoroughly the mixture is briquetted into the desired shape under relatively high pressure, for example, 75,000 pounds per square inch. The articles are placed in a non-oxidizing atmosphere and heated to a temperature and for a time sufficient to cause alloyage of the metallic particles but not to cause fusion of the particles into a solid mass.

During the heat treating operation the copper and tin will alloy to form grains of copper-tin alloy separated by crystals of graphite and by minute cells which remain after the escape of the volatile ingredients.

It has been the practice to pack the articles to be treated in iron or steel pots and cover them with charcoal or the like in order to protect them from the oxygen which may be present in the heat treating furnace.

After the heat treating operation the boxes are removed from the furnace and are cooled to room temperature before the removal of the contents. It is obvious that considerable time is consumed in loading and unloading these boxes and that some heat must be wasted in order to heat the boxes and the packing material as well as the metal articles.

The present invention provides for heating the briquetted articles in a non-oxidizing atmosphere which contains  $\text{CO}_2$  and  $\text{CO}$  and for cooling the articles gradually in a similar atmosphere. In order to carry out this process the present invention provides for heating the briquetted article in a surface com-

100

bustion furnace and for gradually cooling the article in a cooling chamber communicating with said furnace.

Referring to the drawings, numeral 20 designates as a whole the surface combustion furnace which includes a heating chamber 21 into which a gaseous fuel mixture is introduced through pipes 22. The furnace fuel consists of a mixture of air and an atomized 10 or gaseous hydrocarbon fuel which issues from burner nozzles 23 and, when ignited, burns in broken carborundum pieces 24 as is customary in a surface combustion furnace. The rear end of the furnace 20 is provided 15 with an opening 26 which leads into a tubular cooling chamber 27. The combustion products of the furnace which include inert gases,  $\text{CO}_2$  and a reducing gas such as  $\text{CO}$ , will pass into the chamber 27 and also up the stack 28. 20 The chamber 27 is connected with the stack 28 by flue pipe 29. Stack 28 is provided with a damper 30, and pipe 29 with a damper 31. These dampers may be regulated to vary the 25 temperature of the chambers 21 and 27 and also quantity of the combustion products which enter the chamber 27.

A chain conveyor 40, represented by parallel dot and dash lines, is roved around sprocket wheels 41, 42, 43, 44 and 45 and extends along the floors of chambers 21 and 27. The sprocket 44 is the driving sprocket and is driven through a worm wheel 46, a worm 47 and a shaft 48 by a motor 49. The motor is operated so as to cause the chain to move 35 through the furnace in the direction of arrow 50. The articles to be heat treated are placed in trays 51, which are laid upon the conveyor chain.

The chain proceeds through the furnace 40 chambers at a rate sufficient to produce the degree of sintering desired. The articles are heated in chamber 21 to a temperature of about  $1600^{\circ}$  Fahrenheit which is below the fusion point of copper, the metallic ingredient which has the highest fusion point. The temperature and time are sufficient to produce alloyage of the copper and tin while the articles are in the chamber 21. As the articles progress through the chamber 27 from 50 the hottest part to the coldest part they are subjected to the combustion products of chamber 21 which include  $\text{CO}_2$  and  $\text{CO}$ . By the time the trays 51 have passed out of the furnace rear door 52, they will have been 55 cooled to such a temperature that the oxygen in the external atmosphere will have no harmful effects.

After removal from the trays the articles are machined or swaged to the desired size 60 and are impregnated with lubricating oil.

By subjecting the articles to an atmosphere which is entirely free of active oxygen, the temperature may be carried to a higher degree than in furnaces requiring that the articles be 65 packed in charcoal or other similar materials.

Consequently the time of heat treatment may be materially reduced. It is believed that the carbon monoxide tends to reduce the metallic oxide which may be present and therefore facilitates the alloyage of the metallic particles. The carbon dioxide may increase the porosity of the material by reacting to some extent with the graphite. The desired atmosphere within the furnace may be produced by regulating the proportions of 70 fuel and air which are admitted by the pipes 75 22 to the nozzles 23.

A furnace which has been found satisfactory for heating small articles, such as bearings for one inch shafts or smaller, is one having a chamber 21 which is 32 inches wide, 15 inches deep and 6 inches high; and having a cooling chamber 27 provided by a pipe which is 10 feet long and 7 inches in diameter. The diameter of flue 28 is  $4\frac{1}{2}$  inches; and flue 29, 80  $2\frac{1}{2}$  inches. The temperature in the chamber 21 should be preferably from 1500 to 1580 degrees Fahrenheit. The temperature in the cooling chamber 27 will vary from 1100 to 1350 degrees adjacent to chamber 21 to a temperature of from 200 to 300 degrees Fahrenheit at the rear opening 52. Gas analysis of the gases taken from different points in the furnace show that there is practically no oxygen in the chamber 21 and in the portion 90 of chamber 27 near to the chamber 21. At a point near where the pipe 29 joins the chamber 27 the oxygen in the chamber 27 was found to be from 2% to 3%; and to be between 5% and 6% near the door 52. The carbon monoxide was found to vary from 9% to 11% in the chamber 21 to from 3% to 4% near the rear opening 52. The carbon dioxide was found to be present in quantities of 3% to 5% in the furnace and cooling chamber. 100

While the form of embodiment of the invention as herein disclosed, constitutes a preferred form, it is to be understood that other forms might be adopted, all coming within the scope of the claims which follow. 110

What is claimed is as follows:

1. Apparatus for heat-treating articles composed of finely divided metals, and graphite comprising, in combination, a sintering chamber containing surface combustion means for heating said articles in the reducing atmosphere of combustion products of surface combustion, a cooling chamber for said articles in communication with said first chamber, an exit flue leading from said sintering chamber, a branch flue leading from said exit flue to said cooling chamber, and valve means in said flues for maintaining a regulated amount of combustion products in said cooling chamber. 115

2. Apparatus for heat treating articles composed of finely divided metals and graphite, comprising, in combination, a chamber for receiving the combustion products of surface combustion, a non-insulated elongated 120

125

130

cooling chamber in open communication with the first chamber, a passage connecting said chambers and adapted to convey combustion products from the first chamber into the cooling chamber, and means for conveying articles successively through said first and second chambers.

5 3. Apparatus for heat treating articles composed of finely divided metals and graphite, comprising, in combination, a chamber for receiving the combustion products of surface combustion, a non-insulated elongated cooling chamber in open communication with the first chamber, a passage connecting said chambers and adapted to convey combustion products from the first chamber into the cooling chamber.

10 4. Apparatus for heat treating articles composed of finely divided metals and graphite, comprising, in combination, a chamber for receiving the combustion products of surface combustion, a non-insulated elongated cooling chamber in open communication with the first chamber, a passage connecting said chambers and adapted to convey combustion products from the first chamber into the cooling chamber, and means for regulating the flow of combustion products through said passage.

15 30 In testimony whereof I hereto affix my signature.

HARRY M. WILLIAMS.